

UNITE

FICE.

CLINTON P. TOWNSEND, OF WASHINGTON, DISTRICT OF COLUMBIA, ASSIGNOR TO  
GENERAL BAKELITE COMPANY, OF NEW YORK, N. Y., A CORPORATION OF NEW  
YORK.

## COATING COMPOSITION.

1,273,954.

Specification of Letters Patent.

Patented July 30, 1918.

No Drawing. Original application filed November 30, 1909. Serial No. 530,644. Divided and this application filed December 18, 1914. Serial No. 877,874.

*To all whom it may concern:*

Be it known that I, CLINTON PAUL TOWNSEND, a citizen of the United States, residing at Washington, in the District of Columbia, have invented certain new and useful Improvements in Coating Compositions, of which the following is a specification.

This invention relates to coating surfaces, the object of the invention being the provision of a durable protective coating, applicable to all surfaces and particularly to those of iron and steel.

It has been proposed heretofore to protect iron surfaces by precipitating upon them a film of copper or other metal, and to apply varnishes, lacquers, paints and the like to the metallic film so produced. I have found that under proper conditions it is practicable to produce in a single operation, upon conductive surfaces as those of iron, steel or other metals, a galvanic deposit of a coating metal and a protective coating for such deposit. This procedure is highly advantageous, not only by reason of the simplicity of the process, but because on the one hand the conditions of operation result in the production of an unusually adherent, perfect, non-oxidized and permanent film of the coating metal, and on the other hand the presence of this metal results in a better adherence of the protective varnish or coating.

The invention will be described by means of an illustrative example, but it is to be understood that it is not limited to the materials or proportions therein mentioned.

A mixture of a phenolic body, such as phenol or its homologues, and formaldehyde, or a soluble reaction product thereof, is compounded with a suitable solvent possessing the capability of yielding electrolytically conductive solutions of metallic salts; of such solvents methyl and ethyl alcohol, phenol and acetone are examples. To the solution so prepared or to either component thereof, is added a metallic salt soluble in the particular solvent employed. Thus, for example, hydrated or anhydrous cupric chlorid is dissolved in commercial methyl or ethyl alcohol, and the green solution so prepared is utilized as a solvent for the condensation product of phenols and formaldehyde, yielding therewith a dark red or brown varnish which dries

quickly and possesses excellent protective qualities. This varnish remains clear for 55 long periods, is quite permanent in character, and possesses a more or less fluid consistence according to the proportion of solvent and condensation product used. If a non-acid varnish of this character be applied, by 60 dipping, brushing, spraying or otherwise to clean surfaces of iron or steel an almost instantaneous and very striking transformation accompanied by a change of color will be observed, the coating darkening and acquiring a high degree of opacity and luster.

If the iron or steel body coated as above be thereafter partly immersed in alcohol or other solvent for the varnish constituent of the coating, there will be exposed upon the 70 metallic surface a very perfect and integral film of copper, to the unoxidized metallic surface of which film the undissolved portions of the protective coating will be found strongly adherent. The presence of this metallic coat or plating is highly advantageous, in that it not only affords an added protection for the metal against oxidizing or corrosive influences, but it also increases the adherence of the protective coating and renders it more resistant to cracking or scaling. Furthermore the precipitation of copper or 75 other electronegative metal is accompanied in this particular instance by a corresponding formation of iron chlorid, which serves 80 as a condensing agent to accelerate the hardening of the coating.

The coating composition may be slightly acidulated with advantage for certain applications, a small proportion of acid, as for 90 example hydrochloric acid, appearing to result in a quicker deposition of the coating metal, particularly upon slightly oxidized or tarnished metal surfaces; in the use of such acid solutions the rapid darkening 95 above referred to as characteristic of the neutral or basic varnishes is not observed, and the coated surface may present substantially the color due to the precipitated metal; a bright copper-colored coating for instance 100 being obtained with this metal, and a gray metallic coating with salts of tin and lead. In place of copper I may employ salts of all other metals which are soluble in the particular solvent employed and are, in this 105 solution and in presence of the coating mate-

- rial, electronegative to iron or other metal to be coated or capable of precipitation thereon. Metallic salts should be selected whose acid radicals form with the metal to be coated, salts of this metal which are soluble in the solvent employed. For example, iron or steel is advantageously coated with tin and lead from their chlorid and acetate solutions respectively. As a single further illustrative example, I may mention that if mercuric chlorid be dissolved in an alcoholic solution of a condensation product of phenol and formaldehyde, and the resulting varnish be applied to copper, it will be found that the copper has been amalgamated beneath the coating of varnish and that the latter is very adherent and resistant to mechanical or atmospheric influences. Without multiplication of examples, it is to be understood that the method is applicable broadly to the production upon metallic surfaces of a composite coating comprising a metallic film or precipitate and a protective or insulating covering in intimate association therewith. The method is applicable also to the production of composite coatings whereof the coating metal is electropositive to the metal to be coated. In this case however it is necessary to employ either an electric current from an external source, or the so-called "contact" method of precipitation, wherein the metal to be coated is electrically connected with a metal which is electropositive as regards that to be precipitated. In this manner satisfactory deposits of nickel may be formed on iron or copper by precipitation in presence of zinc.
- As has been heretofore pointed out by Baekeland (*Journal of Industrial and Engineering Chemistry*, Vol. I, No. 3, March, 1909), phenols and formaldehyde are capable of reacting, in accordance with the specific proportions employed or in presence of particular condensing agents, to yield a great variety of condensation products, certain of which, and especially those produced in presence of basic condensing agents, are soluble in alcohol, acetone, phenol and similar solvents, but are capable under application of heat of undergoing polymerization, becoming hard, infusible and resistant to all known solvents. I prefer to utilize the valuable properties of these heretofore-described condensation products, inasmuch as it is only necessary to heat the coating in order to effect its transformation into an infusible and insoluble body, in which the metal is indissolubly combined. The invention is not however restricted to the employment of such condensation products; instead I may use alcohol-soluble condensation products of phenols and formaldehyde which are not capable of hardening under the influence of heat (see Baekeland, *Journal of Industrial and Engineering Chemistry*, Vol. I, No. 8,

August, 1909) or I may use such natural gums or resins as are applicable to the preparation of varnishes of the class described.

The compositions above referred to are applicable to the coating of other than metallic surfaces, and possess great advantages for particular uses, particularly by reason of the toxic action of the metallic compounds on living organisms. For example they may be applied to the wooden or metal bottoms of ships, to piling and other submerged structures, and in general in all cases where an anti-fouling composition is applicable. For such uses there may be incorporated and indissolubly combined with the condensation products of phenols and formaldehyde, or with varnishes prepared therefrom, any soluble or insoluble inorganic or organic poison or toxic body capable of preventing or checking the growth or adhesion of barnacles or seaweeds, the attacks of worms or insects, etc. For this purpose the salts or compounds of copper or mercury compounded with those condensation products of phenols and formaldehyde which are capable of transformation under the influence of heat into an insoluble and infusible polymerized product will be found efficient. The liquid or molten condensation products of phenols and formaldehyde are substantially non-conductive, and while they are solvents for certain metallic salts the solutions so prepared are not well adapted for purposes of precipitation. For this purpose it is necessary to add a solvent as above described which affords electrolytically conductive solutions of the salts. For applications or uses not involving precipitation, the solvent may be omitted.

The metallic film produced as above described is precipitated under strongly reducing conditions, not only by reason of the presence of the organic solvent, but because of the presence of such strong reducing agents as formaldehyde and the reaction products of formaldehyde and phenols. Reducing conditions accelerate the separation of the metal and yield an unoxidized, adherent and relatively permanent metallic film, and are therefore highly advantageous. In case natural or synthetic gums or resins are employed in place of the several condensation products of phenols and formaldehyde above referred to, strong reducing agents, as for example formic or other aldehydes, may be added to secure the above-mentioned advantages.

This application is a division of my application Serial No. 530,644, filed November 30, 1909.

I do not claim in this application a composition of matter containing a phenolic condensation product, a suitable solvent, and a salt of a metal which is capable of pre-

70

75

80

85

90

95

100

105

110

115

120

125

130

cipitation upon a conductive surface in the form of a coating therefor; nor do I claim the method of coating electrically conductive surfaces involving the use of such composition; nor do I claim the article resulting from the practice of such method; such subject-matter being claimed in application 530,644, above mentioned.

I claim:—

- 10 1. As a coating composition, a phenolic condensation product combined with a toxic body, and constituting a vehicle therefor.
2. As a coating composition, a phenolic condensation product combined with a metallic compound having toxic properties, and constituting a vehicle therefor.
- 15 3. As a coating composition, a phenolic condensation product combined with a salt of copper, and constituting a vehicle therefor.
4. As a coating composition, a phenolic condensation product transformable by heat into an infusible and insoluble body, combined with a toxic substance.
- 20 5. As a coating composition, a phenolic condensation product transformable by heat into an infusible and insoluble body, com-

bined with a metallic compound having toxic properties.

6. As a coating composition, a phenolic condensation product transformable by heat into an infusible and insoluble body, combined with a salt of copper.

7. As a new article of manufacture, a base for anti-fouling varnishes and paints, comprising a phenolic condensation product indissolubly combined with a toxic body.

8. As a new article of manufacture, a base for anti-fouling varnishes and paints, comprising a phenolic condensation product indissolubly combined with a poisonous metallic substance.

9. As a new article of manufacture, a base for anti-fouling varnishes and paints comprising the product of condensation of a phenol and formaldehyde, with which is combined chemically a poisonous metallic substance.

In testimony whereof I affix my signature in presence of two witnesses.

CLINTON P. TOWNSEND.

Witnesses:

C. W. FOWLER,  
N. P. LEONARD.